

Oct. 14, 1941.

LE ROY M. DEARING  
PHOTOGRAPHIC SOUND TRACK

2,258,976

Filed May 3, 1940



LE ROY M. DEARING  
INVENTOR

BY *Newton M. Parsons*  
*R. Frank Smith*  
ATTORNEYS

## UNITED STATES PATENT OFFICE

2,258,976

## PHOTOGRAPHIC SOUND TRACK

Le Roy M. Dearing, Rochester, N. Y., assignor to  
 Eastman Kodak Company, Rochester, N. Y., a  
 corporation of New Jersey

Application May 3, 1940, Serial No. 333,203

4 Claims. (Cl. 95—2)

This invention relates to sound tracks in photographic film and particularly to a method for producing a sound track in photographic color film.

The production of a dye sound track in reversal color processes is usually carried out in one of two ways. The sound track may be finished in the same manner as the picture area in which case it will be made up of the same dyes as are present in the picture. A second way is to develop the sound track image by special printing methods or by other physical means after reversal in such a way as to use only one dye for the sound image. In this case the dye chosen is usually the one which has the best infra-red absorption in order that the sound reproduction may have the best quality. These methods have the disadvantage that dyes available for color pictures are not good infra red absorbers and give a contrast and maximum density to infra red light that is too low for satisfactory sound quality. In general, dye sound tracks give weak volume as well as poor quality sound on reproduction.

One method of overcoming these objections is to make the sound track of metal or a metallic salt. For example, silver sulfide has been used in the formation of sound images as described in Capstaff U. S. Patent 1,973,463, September 11, 1934, and Mannes and Godowsky U. S. Patent 2,143,787, January 10, 1939. By these methods a sound track is obtained which has satisfactory contrast and whose maximum density transmits little infra-red. The sulfide sound track, however, does not have a clean highlight and this factor has prevented its general use due to the poor quality sound obtained.

It is, therefore, an object of the present invention to provide a novel photographic sound image. A further object is to provide a novel method for producing a sound track in photographic color film. A still further object is to provide a method for improving the high-light quality of a photographic sound track. Other objects will appear from the following description of my invention.

These objects are accomplished by forming the sound track of silver sulfide and silver iodide, thereby eliminating the objectionable features of sound images formed of silver sulfide alone.

In the accompanying drawing, I have shown in flow sheet form successive sectional views of a multi-layer photographic film illustrating the formation of the sound image according to my invention.

As stated above, I secure beneficial results in the formation of a photographic sound track by using a bath which both sulfides and iodizes the sound track. Any sulfur compound which produces silver sulfide upon reaction with silver halide may be used, together with an alkali metal iodide, such as potassium or sodium iodide.

The ratio of iodide to sulfide in the bath may be varied over a wide range of concentrations. 10 With some reversal films that have a high highlight density an entirely satisfactory bath may be obtained from the use of iodide alone. If greater density than that obtainable with iodide alone is desired, sodium sulfide or thiourea may be added to the solution. In this solution, which 15 contains both iodide-forming and sulfide-forming compounds, the presence of the iodide prevents excessive highlight stain while the sulfide builds up the contrast and maximum density to 20 a satisfactory level. The gamma that can be obtained corresponds to that required for good quality sound, being in the neighborhood of a gamma of one.

In the treatment of the silver bromide or silver chloride sound image with the sulfiding and iodizing bath, the sulfide and iodide react in competition with each other. The sulfide reacts immediately and the upper part of the sound track image is usually composed largely of sulfide. 25 30 The iodide penetrates through to the bottom in a slower reaction and most of the image grains in the lower part of the emulsion layer are silver iodide.

Although my invention may be used for the formation of sound images in black and white as well as color films, it is especially well adapted for the formation of sound images in a process such as that described in Mannes, Godowsky and Wilder U. S. Patent application Serial No. 185,700, 35 filed January 19, 1938. In the process described in that application a three layer film having differently sensitized emulsion layers is exposed to a subject and developed to a negative. After negative development the bottom layer of the film is exposed through the support and developed in a color forming developer. The middle layer is then exposed through the support and developed in a second color forming developer and the top layer is finally exposed from the 40 45 50 emulsion side and developed in a third color forming developer after which all silver images are removed.

In my process the sound track formation may be applied directly after the negative development or after any of the three stages of color

development. In a film of the type described in Mannes, Godowsky and Wilder application Serial No. 185,700, it is to be understood that although the preferred sequence of color development steps is that outlined above, the respective layers may be exposed and developed in a different order. For example, the bottom layer may be exposed and color developed, the top layer may next be exposed and color developed and the middle layer may finally be fogged either chemically or by light and color developed. Good results are obtained by forming the sound track image in this method prior to the development of the middle layer.

My invention will now be described by particular reference to the accompanying drawing. As shown therein, a photographic film comprising a support 10 of any suitable material such as cellulose nitrate, cellulose acetate, synthetic resin or paper is coated with successive emulsion layers 11, 12 and 13 sensitive respectively to the red, green and blue regions of the spectrum. This film will ordinarily contain additional filter and subbing layers not shown, especially a yellow filter layer between the emulsion layers 12 and 13 or incorporated in emulsion layer 13.

The first step in my preferred method is to print the sound and picture images in all three layers of the film. This may be done by simultaneous or successive printing steps. The film is then developed in an ordinary black and white developer such as that disclosed in application Serial No. 185,700 to form the negative metallic silver images 14, 15 and 16 in layers 11, 12 and 13, respectively, and a negative sound image 17 in layers 11, 12 and 13.

The bottom layer of the film, which is red sensitive, is then exposed through the support to red light, the sound track area being masked to prevent exposure at this stage. The film is then developed in a blue-green color forming developer such as that disclosed in Mannes, Godowsky and Wilder United States application Serial No. 185,700 to form blue-green positive image 18 in layer 11. Similarly, the top layer is exposed to blue light from the emulsion side and developed in a yellow color forming developer to form positive image 19 in emulsion layer 13. The sound track area is also masked during the exposure of this layer.

The sound track portion of the film is next treated in a suitable sulfide and iodide or iodide bath to convert the positive portions of the sound track area into a silver iodide or combined silver sulfide and silver iodide sound image 20. This may be done by means of an edge applicator such as that described in Mannes and Godowsky United States Patent 2,143,787, or the edge of the film may be immersed in the sulfide and iodide bath so that the picture area of the film is not affected. After formation of the silver sulfide and silver iodide sound image 20, the middle layer picture area is fogged either by chemicals or by light and a magenta positive image is formed in this layer by means of a suitable color forming developer such as that described in Mannes, Godowsky and Wilder United States application Serial No. 185,700. The film is then treated in suitable bleaching and hypo baths to remove all metallic silver and to leave the silver sulfide and/or silver iodide sound image in the sound track area and the dye images 21, 22 and 23 in layers 11, 12 and 13, respectively.

As indicated above, the range of iodide forming and sulfide forming compounds in the bath

used to form the sound track may be varied over wide limits to obtain any desired contrast as well as any highlight and maximum density. Although sulfide and thiourea are generally used for sulfiding, any substance which will react with silver halide to form silver sulfide may be substituted for the sodium sulfide or thiourea. The pH of the solution is controlled by the addition of alkali such as sodium hydroxide to prevent the formation of hydrogen sulfide gas.

The following general formula indicates a suitable range of concentrations:

|                                  |       |        |
|----------------------------------|-------|--------|
| Potassium iodide                 | grams | To 800 |
| Sodium sulfide 9H <sub>2</sub> O | do    | To 400 |
| Sodium hydroxide                 | do    | To 800 |
| Water to                         | cc    | 1000   |

The following specific examples, which are illustrative only, indicate typical formulae which may be used:

*Example 1*

|                  |       |      |
|------------------|-------|------|
| Potassium iodide | grams | 200  |
| Sodium hydroxide | do    | 50   |
| Thiourea         | do    | 20   |
| Water to         | cc    | 1000 |

*Example 2*

|                                  |       |      |
|----------------------------------|-------|------|
| Potassium iodide                 | grams | 200  |
| Sodium hydroxide                 | do    | 50   |
| Sodium sulfide 9H <sub>2</sub> O | do    | 20   |
| Water to                         | cc    | 1000 |

*Example 3*

|                                  |       |      |
|----------------------------------|-------|------|
| Sodium iodide                    | grams | 600  |
| Sodium hydroxide                 | do    | 50   |
| Sodium sulfide 9H <sub>2</sub> O | do    | 400  |
| Water to                         | cc    | 1000 |

In some cases it has been found necessary to use a solution which is nearly saturated with potassium iodide and sodium sulfide in order to produce a sound track having uniform density throughout the sound track area. When the film is dipped into the solution edgewise, the density of the sound track is sometimes less at the top than at the bottom of the sound track area, unless concentrated solutions are used.

It is to be understood that my method is susceptible of numerous variations coming within the scope of the appended claims.

50 I claim:

1. The method of producing a sound track in a photographic film, which comprises printing the sound track image on the film, developing the film to a negative sound image, and treating the sound track area of the film with a combined sulfiding and iodizing bath to form a combined silver sulfide and silver iodide sound track in the film.

60 2. The method of producing a sound track in a photographic film, which comprises printing the sound track image on the film, developing the film to a negative sound image, and treating the sound track area of the film with a combined sodium sulfide and potassium iodide solution to form a combined silver sulfide and silver iodide sound track in the film.

65 3. The method of producing a combined sound track and picture image in a multi-layer photographic film, which comprises printing the sound track and picture images on the film and developing them to a negative, successively exposing separate emulsion layers while masking the sound track area, and developing them in color-forming developers, treating the sound track

area in a combined sulfiding and iodizing bath to form a combined silver sulfide and silver iodide sound track, and removing from the film the metallic silver images formed in the several development steps.

4. The method of producing a combined sound track and picture image in a multi-layer photographic film, which comprises printing the sound track and picture images on the film and developing them to a negative, successively exposing 10

separate emulsion layers while masking the sound track area, and developing them in color-forming developers, treating the sound track area in a combined sodium sulfide and potassium iodide solution to form a combined silver sulfide and silver iodide sound track, and removing from the film the metallic silver images formed in the several development steps.

LE ROY M. DEARING.